# EUROPEAN PATENT APPLICATION

(11) **EP 0 579 365 A2**
(43) Date of publication of application: **19.01.1994**
(21) Application number: 93304141.0
(22) Date of filing: 27.05.1993
(51) Int. Cl.: B22F 3/24

(54) **Method of improving wear-resistance characteristics of a porous metal machine part**

(30) Priority: 27.05.1992 US 889152
(71) Applicant: Yaged, David Peter, Charlotte, NC 28277 (US)
(72) Inventor: Yaged, David Peter, Charlotte, NC 28277 (US)
(74) Representative: Neill, Alastair William

(57) **Abstract**

A method of improving wear-resistance characteristics of a porous metal machine part by densifying the part throughout its thickness. The method includes the steps of ultrasonically cleaning the part to remove impurities from the pores of the part and then drying the part. The part is then exposed to cryogenic temperatures generated by a cryogenic liquid during a period of time. The period of time is divided into three cycles--a gradual cooling cycle wherein the part is gradually cooled from ambient temperature to a temperature of between minus 173 and 212°C; a soak cycle wherein the part is maintained at a temperature of between minus 173 and 212°C; and a gradual warming cycle wherein the part is gradually warmed to ambient temperature. The surface of the metal part is thereafter removed to a depth of from .000254 to .0254 cm to expose a new densified metal wearing surface; and the newly-exposed metal surface is polished.

## Description

### Technical Field and Background of the Invention

This invention relates to a method of improving the wear-resistance characteristics of a porous metal machine part. For purposes of illustration in this application, the machine part is a sintered metal textile spinning or twisting ring of the type which is typically impregnated with oil to provide a low-friction finish capable of withstanding friction generated by a traveler rotating rapidly around the ring under a yarn-induced tension. Such rings are fed from a oil supply. Oil seeps in minute quantities to the surface of the ring through the pores in the metal and provides the low friction finish to the ring needed to reduce friction.

This type of ring has been used for many years. It has a number of serious disadvantages. The oil on the surface of the rings is slung off of the ring as the traveler rotates. The oil, in the form of extremely tiny droplets forming a mist, coats the yarn being processed, the entire textile machine, the floor surrounding the machine and remains suspended in the air where it can be inhaled by nearby workers.

The yarn must be subjected to a downstream cleaning process to remove the oil. The machines must be wiped down periodically, creating oily waste rags which must be properly disposed of. Oily floors occasionally cause "slip and fall" accidents. Of course, the oil, waste rags, oiling cans and repairs to the oiling apparatus all require parts and labor expense. Oily floors can result in violations of health and safety regulations.

Heretofore no satisfactory method has been devised for ring spinning or twisting yarn without using oiled ring.. Prior attempts to surface treat rings to harden them have not resulted in acceptable lengths of service between maintenance cycles. Prior cryogenic treatments which involve dipping the parts to be treated in a cryogenic liquid only treat the surface of the part.

The method presented in this application is a "dry" process in which a cryogenic liquid is used to cool a chamber in which the parts are contained, so that the parts themselves are never contacted by the cryogenic liquid. Extensive testing has demonstrated that the method results in a permanent change in the structure of the metal takes place at the molecular level which can double the life of a spinning or twisting ring without requiring the use of lubricating oil. At the same time, lower operating temperatures and numerous benefits from the elimination of oil also result.

### Summary of the Invention

Therefore, it is an object of the invention to provide a method of treating metal which densifies its molecular structure.

It is another object of the invention to provide a method of treating metal which permits use of the metal in high friction environments without the use of lubricating oil.

It is another object of the invention to provide a method of treating metal which permits the treatment of used, oil impregnated metal parts to transform them into parts which can be used without lubricating oil.

It is another object of the invention to provide a method of treating previously used oil-impregnated textile spinning or twisting rings to transform them into rings which can be used without lubricating oil.

It is another object of the invention to provide a method of treating new porous metal textile spinning or twisting rings to transform them into rings which can be used without lubricating oil.

It is another object of the invention to provide a method of treating porous metal textile spinning or twisting rings to transform them into rings which can be used with lighter travelers.

It is another object of the invention to provide a method of treating porous metal textile spinning or twisting rings to transform them into rings which operate with less energy consumption.

It is another object of the invention to provide a method of treating porous metal textile spinning or twisting rings to transform them into rings which produce higher quality yarn.

These and other objects of the present invention are achieved in the preferred embodiments disclosed below by providing a method of improving wear-resistance characteristics of a porous metal machine part by densifying the part throughout its thickness. The method includes the steps of ultrasonically cleaning the part to remove impurities from the pores of the part and then drying the part. The part is then exposed to cryogenic temperatures generated by a cryogenic liquid during a period of time. The period of time is divided into three cycles--a gradual cooling cycle wherein the part is gradually cooled from ambient temperature to a temperature of between 280 and 350 F.; a soak cycle wherein the part is maintained at a temperature of between 280 and 350 F.; and a gradual warming cycle wherein the part is gradually warmed to ambient temperature. The surface of the metal part is thereafter removed to a depth of from .00001 inches to any depth to expose a new densified metal wearing surface; and the newly-exposed metal surface is polished.

According to one preferred embodiment of the invention, the machine part is a part having oil-impregnated pores, and the method includes the step of ultrasonically-removing the oil from the pores of the metal.

According to another preferred embodiment of the invention, the step of drying the part comprises warming the part in an oven to drive off moisture in and on the part.

According to yet another preferred embodiment of the invention, the step of removing the surface of the metal part comprises the steps of exposing the surface of the part to an abrasive material.

According to yet another preferred embodiment of the invention, the cryogenic liquid is chosen from the group consisting of nitrogen, argon and helium.

According to one preferred embodiment of the invention, the cooling cycle lasts approximately eight hours, the soaking cycle lasts between five and twelve hours, and the warming cycle lasts between five and fifteen hours.

According to another preferred embodiment of the invention, the metal part comprises an oil-impregnated textile machine spinning or twisting ring.

According to another preferred embodiment of the invention, the step of removing the surface of the ring includes the steps of mounting the ring in a rotating fixture, rotating the ring at high speed and engaging the ring with the abrasive material.

According to yet another preferred embodiment of the invention, the step of polishing the part comprises mounting the ring in a rotating fixture, rotating the ring at high speed and engaging the ring with a buffing material.

According to yet another preferred embodiment of the invention, the parts are exposed to cryogenic temperatures in a chamber which is cooled by the cryogenic liquid without contact between cryogenic liquid and the parts.

### Description of a Preferred Embodiment

The method will be described with reference to the treatment of sintered metal spinning or twisting rings. The sintered metal is porous to permit slow movement of oil from within the structure of the ring to the surface for lubricating purposes. Such rings are used on spinning and twisting machines, respectively. Lengths of yarn-forming material are passed around a small C-shaped traveler which is spinning rapidly around an annular surface of the ring. The yarn passes under the rapidly spinning traveler whereby twist is introduced into the yarn. The yarn is immediately thereafter wound onto a bobbin concentrically positioned with reference to the ring. Whether processing previously used or new rings, they are first inspected under a 30X microscope to determine the condition of the ring and to evaluate how much metal will need to be removed from the surface later in the process. The amount of metal to be removed varies with the surface condition of the ring.

Then, the rings are cleaned by placing them in an ultrasonic bath containing suitable cleaning chemicals and water. This ultrasonic process will clean oil and other residue from not only the surface, but from deep within the pores of the porous metal.

The rings are thoroughly dried throughout their structure to remove any cleaning residue, such as moisture. This can be done by "baking" the rings in a warm furnace. This process will drive the moisture and volatiles out of the ring structure, not just off of the ring surface.

After cleaning, the cryogenic process begins. The process utilizes a cryogenic chamber within which the rings are placed. The chamber is cooled by contact with a cryogenic liquid such as liquid nitrogen, argon or helium. There is never any direct contact between the parts being treated and the cryogenic liquid. Therefore, the process is referred to as a "dry" process. This permits very precise, gradual, computer controlled cooling and warming. This is in significant contrast to processes which dip or submerge parts to be treated in the cryogenic liquid. Such a submerging process cools the part so rapidly that cracking or crazing of the part can occur. Furthermore, such processes tend to affect only the surface of the part, rather than the entire structure of the part through its entire dimensions.

The ability to precisely control the cooling and warming cycles permits the characteristics of the parts being treated to be carefully analyzed in correlation with the process parameters and the parameters changed in response to empirical observations and predictions about how changes in the parameters might affect changes in the molecular structure of the parts being treated. The significant parameters are the cryogenic liquid used and thus the temperature to which the parts can be lowered, the rate of change in temperature during the cooling and warming cycles, and the length of time of the soak cycle.

By way of example, a treatment process wherein a quantity of 200 used, previously oil-impregnated rings are treated, utilizes the following parameters:
Cryogenic liquid--180 liters
Beginning temperature-Ambient (approximately 72 degrees F.)
Cooling cycle time period--B hours
Minimum temperature--82°C
Soaking cycle time period (time at minimum temperature--8 hours)

Warming back to ambient temperature cycle time period--8 hours

The cooling and warming temperature occurs at a constant rate of change throughout the range of change. However, the rate of change can be varied based on empirical observations which indicate a desireable variation in the qualities of the treated parts subjected to a differing rate of change. By "variation in rate of change" is meant one or more increases or decreases in the rate of change of temperature during the warming and/or cooling cycles. Of course, the constant rate of change can itself be varied from one treatment process to the next.

Generally, the time to minimum temperature will approximate eight hours. The snaking time will range between five and twelve hours. The warming time will range between five and fifteen hours. The treated rings are characterized by having a denser molecular structure which extends from the surface uniformly through the thickness of the material.

After the treated parts have reached ambient temperature, they are removed from the chamber and inspected again. The rings are loaded one at a time onto a fixture which secures the ring to a rotating table fixture. This device holds the ring stationary while it is rotated. The rotating table fixture can be motor-driven or rotated manually. While the ring is rotated, it is pressed into a rotating Bear-Tex abrasive wheel mounted either vertically or horizontally. A layer of metal skin is removed of about .00001 inches to .010 inches depending on the condition of the ring as determined before the treatment process began. Generally, the abrasive process removes blemishes from the surface of the ring.

After the above surface-removing process is completed, both sides of the ring are again inspected to determine if the surface finish is sufficiently smooth for polishing. If so, the ring is loaded into a second rotating fixture similar to the surface-removing fixture. This time a cotton buffing wheel is used to put a final finish on the ring. A buffing compound is placed on the buffing wheel and then pressed into the rotating ring. A minute quantity of additional material is removed, resulting in an extremely fine, highly polished surface finish. Both sides of the ring are treated in the same manner.

Different types of compounds can be used depending on the finish desired and the Rockwell "C" hardness of the metal part being processed. One suitable buffing compound for use as described above is Tripoli.

This process results in only a very small quantity of metal being removed, thereby not altering the overall shape of the ring. A further inspection process is carried out and then any residual polishing compound is removed. The newly treated rings are ready for packing, shipment to the user and installation.

A method for improving the wear resistance characteristics of a porous metal machine part is described above. Various details of the invention may be changed without departing from its scope. Furthermore, the foregoing description of the preferred embodiment of the invention and the best mode for practicing the invention are provided for the purpose of illustration only and not for the purpose of limitation--the invention being defined by the claims.

## Claims

1. A method of improving wear-resistance characteristics of a porous metal machine part by densifying the part Throughout its thickness, comprising the steps of:
(a) ultrasonically cleaning the part to remove impurities from the pores of the part;
(b) drying the part;
(c) exposing the part to cryogenic temperatures generated by a cryogenic liquid during a period of time divided into:
(i) a gradual cooling cycle wherein the part is gradually cooled from ambient temperature to a temperature of between minus 173' and minus 212°C;
(ii) a soak cycle wherein the part is maintained at a temperature of between minus 173'' and minus 212°C; and
(iii) a gradual warming cycle wherein the part is gradually warmed to ambient temperature;
(d) removing the surface of the metal part to a depth of from .000254 cm to .0254 cm to expose a new densified metal wearing surface; and
(e) polishing the newly-exposed metal surface.

2. A method according to claim 1, wherein the machine part is a part having oil-impregnated pores, and including the step of ultrasonically-removing the oil from the pores of the metal.

3. A method according to claim 1, wherein the step of drying the part comprises warming the part in an oven to drive off moisture in and on the part.

4. A method according to claim 1, wherein the step of removing the surface of the metal part comprises the steps of exposing the surface of the part to an abrasive material.

5. A method according to claim 1, wherein said cryogenic liquid is chosen from the group consisting of nitrogen, argon and helium.

6. A method according to claim 1, wherein the cooling cycle lasts approximately eight hours, said soaking cycle lasts between five and twelve hours, and said warming cycle lasts between five and fifteen hours.

7. A method according to claim 6, wherein said metal part comprises an oil-impregnated textile machine spinning or twisting ring.

8. A method according to claim 7, wherein the step of removing the surface of the ring includes the steps of mounting the ring in a rotating fixture, rotating the ring at high speed and engaging the ring with the abrasive material.

9. A method according to claim 1 or 7, wherein the step of polishing the part comprises mounting the ring in a rotating fixture, rotating the ring at high speed and engaging the ring with a buffing material.

10. A method according to claim 1 or 7, wherein said parts are exposed to cryogenic temperatures in a chamber which is cooled by said cryogenic liquid without contact between cryogenic liquid and said parts.

11. A method of treating a porous metal machine part which includes submitting the part to cryogenic treatment, characterised in that the treatment includes steps of: a gradual coding cycle from ambient temperature to a temperature below minus 173 °C; a soak period during which the temperature is maintained at below minus 173 °C and a gradual warming period back to ambient temperature.

12. A method of treating a porous metal machine part which includes submitting the part to cryogenic treatment, characterised in that the part is exposed to cryogenic temperatures without contact between the cryogenic liquid and the part.
